

# UNITED STATES PATENT OFFICE.

FRANCIS C. FRARY, OF MINNEAPOLIS, AND STERLING TEMPLE, OF ST. PAUL,  
MINNESOTA.

## COMPOSITION OF COPPER ALLOYS AND PROCESS OF MANUFACTURING THE SAME.

1,169,392.

Specification of Letters Patent. Patented Jan. 25, 1916.

No Drawing.

Application filed September 22, 1915. Serial No. 51,984.

*To all whom it may concern:*

Be it known that we, FRANCIS C. FRARY and STERLING TEMPLE, citizens of the United States, and residents, respectively, 5 of Minneapolis, in the county of Hennepin and State of Minnesota, and St. Paul, in the county of Ramsey and State of Minnesota, have invented certain new and useful Improvements in the Composition of Copper Alloys and Processes of Manufacturing 10 per Alloys and Processes of Manufacturing Same, of which the following is a specification.

Our invention has for its object to provide an alloy of copper having certain desirable properties, particularly hardness. 15

In carrying out our invention, we alloy with the copper a metal of the alkaline earths (calcium, barium, strontium and magnesium) and we find that by the use of a 20 very small quantity of the metal of the alkaline earths, the hardness of the copper may be materially increased. As examples of such alloys, we have made alloys of copper containing less than one per cent. of each 25 of the above-named metals, (calcium, barium strontium and magnesium), and find these alloys to make sound castings which are harder than pure commercial copper, and of high electrical conductivity.

30 In making castings of pure copper, it is well known that difficulty is experienced with blow-holes, caused by gases, such as oxygen and nitrogen, which have been absorbed by the molten metal, and are given

off just before it solidifies. It is well known 35 that metals of the alkaline earths have a very great affinity for and combine very rapidly with such gases at the temperature of molten copper: if, therefore, a copper alloy containing such metals be added to the 40 molten copper and thoroughly mixed with the same just before casting the copper, the gases are removed and a sound casting is produced.

It is obvious that in order to secure the 45 desired result at a minimum expense it may be desirable to manufacture or use alloys or mixtures of alloys containing more than one of the metals of the alkaline earths, each of which would produce its share of the desired effect as above explained. 50

What we claim is:

1. As a new article of manufacture, a hard alloy of copper with a metal of the alkaline earths. 55
2. As a new article of manufacture, a hard metallic alloy, containing a main body of copper, and in addition thereto containing a metal of the alkaline earths.
3. As a new article of manufacture, a 60 hard alloy containing copper and calcium.

Signed at Minneapolis, Minn., this 20th day of September, 1915.

FRANCIS C. FRARY.  
STERLING TEMPLE.

In presence of—

HILDA C. JOHNSON,  
ANNA M. McNULTY.